

Aug. 11, 1942.

S. A. COHEN ET AL

2,292,510

METHOD OF MAKING ORNAMENTAL COVERINGS

Filed Aug. 3, 1940

2 Sheets-Sheet 1



INVENTORS  
SAMUEL A. COHEN  
RICHARD L. NEWMAN  
THOMAS LEONARD MORRILL, JR.  
CHARLES D. THURMOND

BY *Charles M. Foye*

ATTORNEY.

Aug. 11, 1942.

S. A. COHEN ET AL

2,292,510

METHOD OF MAKING ORNAMENTAL COVERINGS

Filed Aug. 3, 1940

2 Sheets-Sheet 2

FIG. 4



FIG. 5-



INVENTORS  
SAMUEL A. COHEN  
RICHARD L. NEWMAN  
THOMAS LEONARD MORRILL, JR.  
CHARLES D. THURMOND  
BY *Charles M. Fizer*  
ATTORNEY.

Patented Aug. 11, 1942

2,292,510

# UNITED STATES PATENT OFFICE

2,292,510

## METHOD OF MAKING ORNAMENTAL COVERINGS

Samuel A. Cohen, Berkeley, Calif., Richard L. Newman, Somerville, N. J., and Thomas Leonard Morrill, Jr., Albany, and Charles D. Thurmond, El Cerrito, Calif., assignors to The Paraffine Companies, Inc., San Francisco, Calif., a corporation of Delaware

Application August 3, 1940, Serial No. 351,006

9 Claims. (CL 117—13)

This invention relates to a new kind of ornamental and decorative surfacing, to the manufacture and application thereof to articles, and to floor and wall coverings and other articles ornamented therewith.

### The prior art

A large amount of floor and wall covering has been and is being manufactured of the felt base type. This type comprises a base of felt, usually somewhat similar to roofing felt but of a somewhat more dense character, saturated with an asphaltic compound often having a softening point of about one hundred fifteen degrees to one hundred seventy degrees Fahrenheit (115° to 170° F.). A composition made of a drying oil and ester gum, and possibly other compositions also, have been proposed to replace the asphalt. Such felt base coverings usually have a patterned surface, the pattern being applied in commercial operation by a system known as block printing. Ribbed wood blocks are used, and so-called print paints are supplied automatically to the ribs of the blocks by rollers which are in turn automatically supplied with the paint. Each block receives its required color and applies it to the base, the surface of which is first treated or covered with material to prevent the asphalt of the base from bleeding into and discoloring the applied print paint.

A continuous sheet of prepared felt base material passes through the printing machine, it being stopped to permit the blocks to move downwardly thereonto to apply the print paint, one color at a time. The sheet moves forwardly while the print paint is being applied to the blocks, and finally emerges, with the complete pattern printed thereon from the printing machine, whereupon it is hung in festoons or laid in cut lengths on horizontal racks in a heated room to dry the paint thereon. The different applied colors generally contact each other in the finished product unless the pattern is an open one. Printing presses for this purpose are well known and their structure forms no part of this invention.

The conditions of operation are such that the paint used for printing must have a combination of characteristics not possessed by ordinary paints for successful commercial mass production, and it was necessary to develop a special type of paint, known as print paint for this purpose.

In printed felt base floor and wall coverings the pattern comprises only a thin layer as distinguished from linoleum in which the pattern extends through many times the thickness that it does in the printed felt base covering material.

For successful commercial production there have been certain requirements as to the characteristics of the paint used for printing. It must have the property of "leveling" without "flowing"

so that the whole surface of the pattern, including the dividing lines between the different colors will be level without the paint of one color flowing into that of another color.

5 The maximum quantity of the oil which may be used in the print paint is limited by several factors inclusive of the desired hardness of the finished product; the minimum is determined by the desired absence of brittleness.

A good "gloss" has been demanded in the finished product after it has been dried. This property of glossiness depends in part on "pigment volume," that is, the ratio of the volume of the pigment used to the volume of all non-volatile fluid or liquid ingredients used in the print paint. Gloss depends also on the particular oils used, the kind and amount of the resins, and the process by which all of these have been treated. It depends further on the degree of oil absorption by the pigment, the amount of volatile constituents, and possibly on other factors as well.

The "oil length" of a print paint vehicle is the number of gallons of non-volatile oil used therein for each one hundred (100) pounds of resin therein, and is generally about seventy (70) gallons. This oil length may drop as low as thirty (30) gallons at the extreme, but brittleness will appear at or about this low a limit. Normally it should not exceed one hundred (100) gallons by any material amount as the necessary hardness and toughness of the dried film may fall off rapidly thereabove.

The wet print paint must not soften too much on exposure to high temperature such as occurs during the drying of the paint, and it must not soften when dry in a hot climate in which the finished article is used.

40 "Temperature susceptibility" depends to a great degree on the type of resin used and upon the oil length. There are certain resins which impart hardness at room temperatures to dried print paint and give good gloss and which are alkali-resistant, but the dried film made from print paints containing these resins is apt to be too brittle when cold and too soft when warm.

45 "Absence of sag" depends, at least in part, on a certain amount of "reactivity" between the vehicle and the pigment. Without sufficient reactivity the paint, no matter what the applied thickness thereof may be, will run similarly to, but perhaps not as fast as, water; and thus it will sag so that the printed figures will run together during the time the floor covering is being lifted vertically to the top racks in the building where they are to be dried; particularly since the material, to meet manufacturing exigencies, is sometimes stopped in this vertical position for two or three minutes during its travel to the drying racks. In some cases too great a degree of "reactivity" between the pigment and the oil

may cause the paint to be "sticky" so that it will not separate quickly and completely from the print blocks during the printing operation, even though the paint may have the proper leveling characteristics.

Ordinary pigments may be used, such, for example, as combinations of zinc oxide, lithopone, barytes, whiting, ochres, iron oxide, lithol red, chrome green, Prussian blue, lamp black, and the like. In addition to the relations given above concerning the volume of the pigment to the volume of the non-volatile fluid ingredients, the combined weight of the pigment used should be about sixty percent (60%) of the paint exclusive of the volatile material therein.

There should be no "residual flow" in the drying racks due to the heat used for drying. This characteristic depends on the resin and on the solvent used, as well as on the driers and the reactivity. Not only should the drier be chosen with respect to the lack of residual flow, but "non-skimming" driers are essential because a good print paint must dry from the bottom up or throughout and it must not form a surface skin first.

The characteristic of "settling of the pigment" depends on the reactivity between the pigment and the oil. The print paint must have enough "set" so that the pigment will not settle out in containers holding the stock paint ready mixed for use on the press, nor in the color boxes of the printing press, yet it must be sufficiently limpid so that it can be properly applied by transfer rolls to the printing blocks, be properly acted on by the doctors, and be properly printed by the blocks.

Even though the print paint must be limpid as just described, yet it must not "stick" to the blocks and form "strings" when the blocks pull away from the base to which the printing is being applied, since such strings are apt to fall back onto the pattern and mar it. It may be noted here that a paint can be made so sticky as to cause the goods being printed to be lifted up by the printing blocks as the latter are withdrawn upwards after making the impression. Too great a reactivity between the pigment and the oil, particularly if the oil contains free acid which is too active, may result in sticking and stringing, and if the stickiness is sufficiently great, in causing the goods to adhere to the printing blocks.

In general it may be said that the type of reactivity sought is one which produces the proper amount of thixotropy but which does not produce stickiness.

"Alkali resistance" should be such that the finished product can be washed with ordinary washing soap or cleansing compounds when it becomes dirty without spoiling it.

In short, a good print paint for use in making conventional floor, wall, and other coverings must be such that it can be printed by means of a flat bed press with the use of a ribbed print block, that a baked (dried) coating of the print paint of sufficient thickness is obtainable, the baked coating having a smooth surface obtained through leveling of the paint after printing, the successive areas being free from stringing, free from bad "block joinings," the paint being of limited flow with absence of sag, and having a baking period of from three to four (3 to 4) days at one hundred sixty degrees Fahrenheit (160° F.), and when baked having the characteristics of toughness, hardness throughout the film,

sufficient flexibility, and elasticity so that, when used as a floor covering it will permit of walking thereon without becoming cracked or otherwise marred or spoiled, gloss, and resistance to wear, to water and to usual soap or washing compounds.

It is not possible to produce or modify all the characteristics of a print paint singly by the mere use, omission, or modification of a particular ingredient, because the change of one component may effect a change in several characteristics; and it is therefore not a simple matter to develop a good print paint.

With all this in view, the various print paint components, the relative proportions thereof, and the functions thereof, must be so co-ordinated as to produce the desired group of print paint characteristics. It will thus be apparent that "print paints" are somewhat akin to printing inks in their functions and somewhat akin to varnish enamels in their ingredients; and that they form a highly specialized class of paints having special characteristics and requiring special ingredients and treatments in the manufacture thereof; and that they are very different from conventional paints for general use. Print paints have been developed in the course of time that meet the requirements rather well, to a greater or lesser extent. Print paints can be printed without first drying with different colors so closely adjacent each other that they contact each other in the finished product with a sharp color boundary line between them, and furthermore, wet print paint can be printed onto wet print paint which has been previously printed, all without smearing.

A description of a typical example of a print paint and how to prepare it follows, all the parts indicated being by weight.

A heat bodied oil of approximately H viscosity on the Gardner-Holt scale may be used, and such oil may, for example, be linseed oil bodied, that is thickened, at five hundred sixty degrees Fahrenheit (560° F.); a varnish of approximately C viscosity on the same scale may also be used, and this may consist of

|                                                                                                                                     | Parts |
|-------------------------------------------------------------------------------------------------------------------------------------|-------|
| Phenolic resin                                                                                                                      | 100   |
| Drying oil                                                                                                                          | 50    |
| V. M. & P. naphtha                                                                                                                  | 100   |
| V. M. & P. naphtha being varnish makers' and painters' naphtha, a designation and a material well known in the art and in commerce. |       |

A vehicle is made, which may consist of

|                     | Parts |
|---------------------|-------|
| Bodied oil as above | 70    |
| Varnish as above    | 30    |
| V. M. & P. naphtha  | 5     |

A base paint is made, which may consist of

|                                    | Parts |
|------------------------------------|-------|
| Lithopone of medium oil absorption | 150   |
| Zinc oxide                         | 50    |
| Vehicle as above                   | 75    |

The final print paint is made of

|                     | Parts |
|---------------------|-------|
| Base paint as above | 100   |
| Vehicle as above    | 40    |

What precedes describes the prior art manufacture and problems involved therein, of felt base floor and wall covering having a patterned ornamental surface in different colors with the different colors generally contacting each other and having common boundaries, each color having a thickness, toughness and other characteristics to make it resistant enough to wear, for

example by people walking thereon, to be desirable from an economic point of view.

The thickness of the colored print paints in the completed product as ready for use is at least about fourteen (14) times that obtainable in the early stage of the floor covering art where isolated narrow lines or small dots were printed in a single color by zincograph rolls or by transfer rubber or gelatine rolls, an example thereof being the printing of imitation wood graining on a background having a color approximating that of wood. Such patterns were necessarily open patterns, that is a multiplicity of isolated narrow lines or small dots were used to make the pattern, with the background showing at unprinted areas. The print paint as described above normally dries after printing to a thickness of five to seven thousandths (0.005 to 0.007) of an inch.

Closed patterns, that is those the individual colors of which collectively formed a thick, continuous surface of substantially the same thickness throughout and without objectionable ridges or depressions at the boundaries between the colors were not possible with the color material used during the early stages of the art, but such products capable of long wear are possible when made of what is known as print paint, even though the background is completely covered by the pattern.

The demand has been for ornamental surfaces which are substantially level throughout, long wear resisting, and glossy; and present day print paints which wear well in the finished product impart a high gloss thereto. There is at least an incipient demand for floor coverings having all of the desirable qualities of those made by present day practice, with the glossiness softened without merely appearing dull. Long research might perhaps develop a print paint suitable for the purpose but manufacturers operating under mass production methods, amounting now to about one hundred fifty-five million (155,000,000) square yards of felt base floor covering per year, are not prone to make any changes in production practice which would be uncertain and experimental. Experimental manufacture would be required if any new material were adopted in place of the present print paint in order to determine what difficulties in manufacture, if any, were caused by it and how the new product would hold up under actual conditions of use. Furthermore, long research would probably be required, with no certainty of success, to develop a suitable print paint which would not be glossy and still impart a pleasing appearance, because any change to modify a characteristic would result in changing other characteristics.

#### The invention

Objects of this invention are:

To modify the appearance of products printed with material characterized as present day print paint; to control, modify, or lessen the glossy finish thereof; to modify the structure of and strength of the applied paint coat; to make the paint coat thicker and more wear resistant in the finished product than that printed on; to provide printed felt base covering material which will have a more linoleum-like appearance and greater resistance to wear than conventional printed felt base covering material; to produce a pleasing, smooth-looking finish which is neither glossy nor flocklike but which may be characterized as intermediate therebetween, and which is not glossy nor coarse nor having a flat or opaque

appearance which may be characterized as soft and velvety but without any appearance of the velvet nap; to produce a pleasing appearance like that of a top plan view of a perhaps hypothetical material having a short nap of vertically upstanding fibers which are so short, fine, and closely adjacent to each other that said top plan view thereof does not appear absolutely uniform and yet the individual fiber ends are not individually visible to the eye; to produce a pleasing appearance similar to that of a paint surface having a very large number of very small protuberances or slightly raised dots very closely adjacent each other and thus having a "softer" appearance than a glossy level paint surface. Another object is to provide simple, economical, commercially feasible methods for accomplishing the above objects; to accomplish the above objects without any necessity for changing the print paint now used in the production of the glossy product; and other objects will become apparent on reading this specification in connection with the accompanying drawings which form a part hereof.

Such drawings are principally diagrammatic or schematic in nature and the different parts thereon are shown out of their true relative proportions.

Fig. 1 is a schematic view of the preferred apparatus, with some parts in section;

Fig. 2 is a similar view of a modification of a part thereof;

Fig. 3 is a similar view of another modification of the same part;

Fig. 4 is an approximate end view of a product made according to this invention; and

Fig. 5 is a similar view of another product made according to this invention.

The preferred method of making the novel product will now be described with reference to Fig. 1 of the drawings. The methods of making the felt base, of treating it with seal or other coats, and thereafter printing the various colors of the pattern thereon are the conventional ones used in the manufacture of present day printed felt base floor and wall coverings. Before the print paint forming the pattern has dried, and preferably just after the printed sheet 11 emerges from the printing machine 13, wood flour is applied to the wet paint surface. This is preferably spruce wood flour of the following screen analysis wherein "Tr." stands for trace, this flour to contain no coarse particles.

|                            | Screen mesh | Maxi-       | Mini-       | Average     |
|----------------------------|-------------|-------------|-------------|-------------|
|                            |             | Mesh        | Percent Tr. | Percent Tr. |
| Proportion remaining on... | 65          | Percent Tr. | 0           | 0           |
| Proportion remaining on... | 100         | Tr.         | 0           | Tr.         |
| Proportion remaining on... | 200         | 25          | 15          | 20          |
| Proportion remaining on... | 325         | 45          | 35          | 40          |
| Proportion passing thru... | 325         | 45          | 35          | 40          |

Thus, practically all of the wood flour passes through a one hundred (100) mesh screen; substantially fifteen percent (15%) to twenty-five percent (25%), with an average of substantially twenty percent (20%) thereof remains on a two hundred (200) mesh screen; substantially thirty-five percent (35%) to forty-five percent (45%), with an average of substantially forty percent (40%) thereof remains on a three hundred twenty-five (325) mesh screen; and substantially thirty-five percent (35%) to forty-five percent (45%), with an average of substantially forty percent (40%) passes through the last mentioned screen.

The sheet 11 passes over the roller 15 to form a loop 17 and then over the roller 19, this loop being provided to allow sufficient slack since the sheet moves intermittently out of the printing machine while thereafter it moves at constant speed. The roll 15 is power driven at constant speed but is of such a nature that it will slip under and in contact with the sheet when the latter is not in motion. The roll 19 is power driven at constant speed, there being sufficient friction between this roll and the sheet so that the loop 17 and the next loop to be hereinafter referred to are maintained without either one straightening out.

The first application of the wood flour is best only a light application lightly applied, just enough being applied to "set" the surface of the wet paint, that is to make it less fluent to prepare it for a heavier application of the wood flour. This setting merely amounts to making the surface of the wet paint less "wet" or fluent. The most expedient way to accomplish the first and light application is by floating it in air (or other gas if desired), making what might be termed a cloud or fog of wood flour, and directing such cloud or fog onto the wet, printed surface. For this first application of the wood flour, a conduit 21 is provided to direct the air laden with the wood flour onto the freshly painted surface and across the whole width of the sheet as it passes over the roll 19. The cloud or fog should, of course, not have sufficient force to disturb the painted surface, but it should have sufficient velocity so that particles of flour reach all parts of the paint surface evenly and become fixed therein. A very uniform mixture of air and flour should be used to prevent the flour from forming flocks or bare spots on the paint surface. The angle at which the air-wood flour mixture strikes the paint may be about thirty degrees (30°).

Naturally, there will be an excess of wood flour which does not adhere to the paint and such excess is blown into a trough 23 from which it is removed through one or more pipes 25 by means of suction applied thereto. The sheet then forms another loop 27 by passing over the roll 29, the loop 27 containing a mass of the wood flour 31 in such an amount that there will be a relative movement between it and the sheet which may be described as sliding rather than merely rolling or tumbling. With the two vertical portions of the loop 27 about twenty (20) inches apart and this loop at least several times as deep, the thickness of the wood flour layer therein may range from about one (1) inch up to five (5) or six (6) inches.

Roll 29 is power driven at constant speed and has the same peripheral speed as the roll 19, and it may be of the same diameter. As the printed sheet carrying the wood flour passes over the roll 29 it is brushed by means of a very soft revolving brush 33 which preferably rotates in a direction opposing the movement of the sheet and is preferably made of long, soft goat hair or the like. Other hair coverings may be substituted, such as beaver, but not sufficient advantage is gained to offset the cost of this expensive fine fur. The long, soft hair bristles push the wood flour down into the paint layer without there being any evidence of smearing if the speed of the brush is properly chosen. The proper speed will depend on the length and the softness of the bristles and perhaps on other factors, and it is best ascertained once and for all by trial.

The hardness, or harshness, of the bristles may be the greater, the greater is the amount of wood flour imbedded in the paint, because the greater the amount of the wood flour therein the greater will be the resistance it offers to displacement.

Any excess of wood flour which is not pushed down into the paint layer by the brush will be removed by it from the surface and thrown into the trough 35 from which it may be removed through one or more pipes 37 to which suction is applied. It is preferred not to let such removed excess wood flour drop back into and mix with the wood flour within the loop 27, since there may be times in large scale manufacturing when this removed wood flour may have acquired characteristics unsuitable for the production of the best product. The sheet then forms the loop 39 to take up any slack not otherwise provided for in the process.

All of the parts so far described about which wood flour flies about are preferably within an enclosure 41 forming a substantially sealed chamber except for slots 49 and 51 to permit the ingress and egress of the sheet, and if desired the loop 17 may also be within such enclosure. The treatment with the wood flour is the only deviation from standard practice in the manufacture of printed felt base floor and wall coverings, in the process so far described, which, as already stated above, have been manufactured on a very large scale. The next steps to which the sheet is subjected are the old conventional ones of cutting into lengths as desired, and drying the paint to harden it. The sheet passes onto a vacuum belt 41 which is endless and passes over rollers 43, 45 at least one of which is to be driven at the proper speed. This belt advances the sheet to the cutting station at which the conventional knife 53 which has been used for cutting the well-known prior printed felt base floor and wall coverings into lengths is stationed, and it may be used in the same manner and for the same purpose in the manufacture of the product of this invention. The conventional treatment then has been to dry and harden the printed paint on the printed felt base floor and wall coverings by placing the sheets, cut into suitable lengths at the cutting station 53, in horizontal position with the printed face up, on horizontal racks in a suitably heated drying chamber, as set forth in the patent to Rosener, No. 1,743,397, dated January 14, 1930. The same drying chambers and the same method of hardening the paint with the wood flour therein may be applied to the new product. Another way of drying the printed paint is to hang the sheet in festoons which may be stationary or slowly moving in a suitably heated drying chamber which is preferably very high to permit of long festoons. Such a drying chamber is indicated at 55 in which are sufficient rollers 51 at a sufficient height above the floor to make the festoons sufficiently long to cause the paint to be thoroughly dried and solidified when the sheet emerges from the chamber.

The subsequent steps of the process depart from prior procedure.

The sheet is next abraded in any suitable manner to loosen and remove excess wood flour on the surface thereof. The degree of abrasion should be sufficient to loosen any excess which might mar the appearance of the product, yet it should not be sufficient itself to mar it. The preferred manner of abrading is by a "self-sanding" operation in which two faces having the

wood flour thereon are caused to rub against each other. With this in view, the sheet is caused to pass in both directions, face to face, between opposed rolls. The surface of contact may be increased by curving the path of the double sheet about one or more of the rolls. One example of how this may be accomplished is by staggering and offsetting the rolls. The dried sheet passes to the right, with the ornamented face up, between rolls 59 and 61, then between the rolls 61 and 63, then over roll 65 by which the direction of the sheet is reversed, the sheet then returning to the left, whereupon it passes between the rolls 61 and 63 and then between the rolls 59 and 61, with the ornamented face downwardly and against the upwardly facing ornamented surface passing to the right. The roll 63 may be omitted, and if desired, the roll 61 also, provided the abrasive effect is sufficient to remove enough of the wood flour to give a pleasing appearance to the ornamental surface and to prevent enough wood flour remaining so that the surface will not have the appearance of flock or of flock-printing.

Any loose particles are suitably removed after the abrading step, preferably by means of suction applied through a hopper-like member 67.

On leaving the roll 59 in its passage to the left as shown on Fig. 1, and after removal of the loose wood flour, the product is complete for some uses except for possible cutting into suitable size, if it has not already been so cut. It shows the printed pattern clearly yet it is not glossy even though a print paint was used which would produce a glossy finish without the use of the wood flour. The appearance is not flock-like but is smooth and homogeneous; and while it is more like that of linoleum than is that of the prior conventional printed belt base covering material, it is even more pleasing than that of linoleum. Its appearance is not coarse nor flat nor opaque like a bright surface which has become scratched or worn, but it is soft and velvety without any nap being visible or present, and it approximates the top plan view of the perhaps hypothetical material having an extremely short nap of vertical upstanding fibers which are so fine and closely adjacent each other that while said view is not absolutely uniform in appearance, yet individual non-uniformities are not apparent.

While the printed decorative pattern has a substantial thickness in the conventional printed felt base floor and wall coverings as made by present day conventional methods, it is still thicker in the product of this invention because the same amount of the same kind of print paint is applied in the same way as formerly, and the immersing of the wood flour thereinto raises the level thereof. The ornamentation is thus made thicker than formerly without the necessity for using more print paint. Not only is the ornamental layer of print paint thicker, but it is more resistant to compression and to wear on account of the solid wood flour imbedded therein. The print paint colors show clearly in spite of the presence of the wood flour, and the color of the wood flour itself is invisible if flour of the proper wood be chosen.

When the product is to be used as a floor covering, or for certain other purposes, it is preferable to apply to the so far completed decorative surface a protective coating of tough, hard, flexible, clearly transparent, waterproof, soil resistant, washable material, which should contain no pigment or anything that hides the pattern or the

5 colors of the pattern, although adjustments or changes may be made in any of these characteristics for special requirements. This coating material may be a varnish or lacquer made up of nitrocellulose, a solvent and a plasticizer therefor; and it may be the coating material ordinarily applied as a coating to ordinary linoleum.

For applying such a coating, the sheet, after leaving the roller 59 for the second time, may be carried over a roller 71 and under a sprayer 73 to which the coating liquid is supplied, and which sprays it onto the decorative surface where it dries.

15 The method of and means for applying the wood flour to the wet printed paint may be varied. For example, the fogging on of the wood flour, that is applying it while floated in a gas may be omitted, as illustrated on Fig. 2, or it may be substituted by another method of application 20 as illustrated on Fig. 3, but with less satisfactory results. The mild, light, preliminary application, as accomplished, for example, by the fogging operation, to give a preliminary set to the wet paint, lends itself peculiarly to the mass production of a product in which the proportion of 25 artistically unacceptable material is a minimum and is increased by elimination of the preliminary light set of the wet printed pattern.

On Fig. 2 the sheet 11 is shown as issuing from 30 the printing machine 13 to a roll 15 and then to a roll 17 to form a loop 79 between them, there being wood flour 81 therein similarly as in the loop 21. Here again there is a relative motion 35 between the sheet and the wood flour 81 which, as in the loop 21, is more in the nature of sliding than rolling or tumbling. A brush 83 similar to the brush 33 performs the same function at the roll 17 as does the brush at the roll 29. A trough-like shield 85 may be provided, the upper part 40 81 of which houses the brush, while the lower trough-like part 89 catches the brushed off wood flour which may be removed from the trough 45 in any suitable manner or it may be accumulated therein if desired. After leaving the parts of the apparatus shown on Fig. 2, the sheet forms a loop 39 and then travels on the belt 41 and past the cutting means 53 as shown on Fig. 1, which 50 may be used if desired, and then to the drying and abrading means shown on such figure, and if desired, also to the coating means shown thereon.

On Fig. 3 the sheet 11 is shown as issuing from 55 the printing machine 13 and passing over rollers 91, 93 and 95 to form the loops 97, 99, both of which contain wood flour 101 and 103 respectively, similarly to the loop 21 on Fig. 1 and the loop 79 on Fig. 2, the relative motions of the wood flour with respect to the sheet being the same as that already described with respect to those figures. A means is provided to remove wood flour loosely adhering to the surface after application, and this may comprise a tapping bar 105 having pivotal connections 107 reciprocated fast by means of an eccentric 109. Any other suitable means for tapping or jarring the sheet may be used. A brush 111, similar in its function to the brushes 33 and 83, is located in the same relative position as indicated in Figs. 1 and 2, with a trough-like member 113 surrounding the brush to catch the thrown-off wood flour which may be removed therefrom by a current of air through a pipe 115. An air blast may be provided to prevent any of the thrown-off wood flour from falling into the loop 99, and this

air blast may issue, for example, from a perforated or slotted pipe 117 extending across the sheet. After leaving the parts of the machine shown on Fig. 3, the sheet forms a loop 39 and then travels on the belt 41 and past the cutter 53 as shown on Fig. 1, if the cutter is to be used. The sheet then passes to the drying and abrading stations shown on Fig. 1, and then, if desired, to the coating station 73 shown thereon.

Fig. 2 illustrates a means and method wherein there is no preliminary application of wood flour prior to the main application. Fig. 3 illustrates a preliminary application prior to the main application, but this preliminary application is considerably heavier and may not be controlled as easily as the application by fogging as shown on Fig. 1.

The brushes 33, 83 and 111, by their very light or mild brushing action, have the function of pushing the applied wood flour down into the layer of wet printed paint and also of removing the excess from the surface thereof without smearing the print paint. In place of the brush any suitable means may be provided which performs both of these functions, either simultaneously or consecutively, and in certain cases means may be substituted which perform only the function of pressing the wood flour down into the layer of printed paint without removing the excess from the surface. The combined effect can be obtained by any light mild rubbing action, preferably with a soft and yielding material. It is preferable, however, to remove excess wood flour from the surface both while the print paint is still wet and after it has dried. Different methods and apparatus for removing the brushed-off excess wood flour and different devices for doing so are illustrated on Figs. 1, 2 and 3, and these or equivalents thereof are interchangeable in the various modifications.

Sprinkling the wood flour onto the print paint, for example in a manner similar to that described in the British patent to Schloesser, No. 692 of 1881, will produce not only uneven distribution, but a flock-like markedly fuzzy surface, as tests have shown, even with the use of the modern print paint which was unknown at the date of said patent.

Sliding the wood flour over the wet print paint pattern, as is done in the loops 27, 79, 91 and 99, produces a smoother and generally more desirable appearance in the finished product than sprinkling the wood flour thereon, and the application is much more uniform than by sprinkling.

The preliminary light application of wood flour to "set" the surface of the paint aids materially in the production of the best high grade product, but it is within the scope of this invention to omit it in such cases where its effect on the finished product may not be essential. It prepares the surface uniformly for wood flour to slide thereover in the loop so that such sliding which has a very mild and light rubbing action, will produce a smoother and more uniform effect. The sliding of the wood flour aids in causing removal of excess wood flour so that the sliding itself makes for uniformity. While the sliding is preferably for the best high grade products, yet it is within the scope of this invention to omit it in such cases where its effects on the finished products may not be essential.

Removal of excess applied wood flour, both before and after the print paint dries, makes for smoothness and aids materially in the production of the best high grade products. It is with-

in the scope of this invention, however, to omit such removal before or after the paint dries, or to omit both, in such cases where the particular effects on the desired products may not be essential. The preferred product is, however, made by the procedure illustrated on Fig. 1 and without the omission of any of the valuable steps described hereinabove.

The natural or non-artificially colored flour of spruce wood is preferred because, of the woods easily available in certain sections of this country, it changes the applied printed colors very little and because such wood is easily converted into a flour having the screen analysis previously indicated. The flour of Ponderosa pine and of slash pine may also be used, as may the flour of other woods if of suitable color or if the characteristics they may impart to the decorative coating are desired. The screen analysis of the wood flour above referred to has been found suitable and is preferred for commercial production on a large scale because it makes a product of excellent appearance. Products may, however, be made according to this invention with wood flours of different screen analyses, but there is danger of materially increasing the proportion of product which will be unsatisfactory from an artistic point of view and therefore subject to rejection. The use of a wood flour which passes through a one hundred fifty (150) mesh screen, the major proportion of which is retained on a slightly finer screen, results in a fairly good product but one which is not as good as that made with the wood flour of the preferred screen analysis. The use of a wood flour passing through a fifty (50) mesh screen, the major proportion of which is retained on a slightly finer screen, does not result in a satisfactory product.

The preferred products are approximately illustrated, much enlarged, with the parts not necessarily in their true proportions, on Figs. 4 and 5, it being impossible to illustrate them more exactly because of the small dimensions involved. The product illustrated on Fig. 4 comprises the conventional saturated felt base backing 141 (shown broken away), the conventional layer or layers of seal coats 143, 145 thereover, and the printed layer of print paint 147 on the seal coat and containing the particles 149 of the wood flour. The product illustrated on Fig. 5 is the same as that shown on Fig. 4 but includes the protective coating 151 applied at 13 on Fig. 1. The particles of wood flour are shown as within and almost throughout the layer of wet print paint. It is not known, however, just how closely adjacent the wood particles are to each other or how far down in the print paint layer they may be. It is known, however, that wood flour particles are imbedded in the dry print paint layer. The colors of the dry print paints having the wood flour applied thereto according to this invention show almost and practically as clearly and brightly as if the wood flour had not been applied, there being practically no instances where loss of brightness or hiding of the color by the wood flour are of an objectionable degree. The wood flour causes the surface to have an almost infinitesimal roughness which is apparent to the eye by its softened appearance. The low color loss, if any, due to the presence of the wood flour, and the soft appearance of the surface apparently indicate that very little, if any, of the wood flour particles project above the dry print paint surface and

that the predominant parts, if not all, of the wood flour particles are imbedded in the dry paint layer, with at least a large proportion thereof just at, but below the surface. The wood flour particles are preferably each in direct contact with the print paint in which they are imbedded but the resulting appearance is quite different from and superior to a product made by mixing the wood flour into the print paint, printing with such a mixture and then allowing the print paint in this mixture to dry. The fine particles of wood flour agglomerate when it is attempted to mix them with print paint of the type herefore described, with the result that the dried surface does not have a uniform appearance. The products of this invention do have a uniform appearance which however is not to be described as absolutely smooth but more in the nature of being very finely and mildly grained like a mat-surfaced photograph. Very little, if any, part of the wood flour particles project above the dried print paint, due to the print paint or the vehicle thereof being absorbed into the wood flour by capillary action, and also to the removal of the excess wood flour from the surface of the dried print paint. The mat effect gives the product not having the above described protective coat thereon a soft, chalky appearance, that is the pattern appears as though it had been made with colored chalk. The product having the above described protective coating thereon shows mild highlights in certain lights, and it still has somewhat the appearance of a mildly mat photograph even though the protective coating may add some gloss.

Figs. 1, 2 and 3, which are diagrammatic or schematic to a great extent, illustrate the principles involved in the making of the product.

Certain more or less specific features have been referred to for the purpose of illustrating this invention, which do not necessarily limit it. It is therefore to be understood that equivalent means and method steps may be substituted for various means and method steps, even though no mention of such substitution may have been made previously hereto in this specification.

The term "print paint" is used in the claims as referring to decorative coating compositions of the general type previously referred to.

We claim:

1. The method of making ornamental printed felt base covering material, which consists essentially in printing a pattern of different touching colors onto a suitably prepared felt base backing with print paint, treating different colored touching portions of the wet printed pattern simultaneously to produce a light application of very fine wood flour of suitable color to the surface of said printed paint to "set" said surface, treating different colored touching portions of the "set" surface simultaneously to a heavier application of said wood flour, moving said wood flour into said paint and removing excess thereof from said surface, drying said wet print paint, and removing excess wood flour from the surface of 65 the dry print paint.

2. The method of making ornamental printed felt base covering material, which consists essentially in printing a pattern of different touching colors onto a suitably prepared felt base backing with print paint, treating different colored touching portions of the wet printed pattern simultaneously with a fog of very fine wood flour to produce a light application of said flour thereto to "set" the surface thereof, sliding wood flour of 75

a similar type over different colored touching portions of said "set" surface simultaneously, lightly rubbing the resulting surface to move said wood flour into said paint while removing excess wood flour from said surface, drying said wet print paint, and abrading excess wood flour from the surface of the dry print paint.

3. The method of making printed felt base covering material, which consists essentially in printing a pattern of different touching colors onto a suitably prepared felt base backing with print paint normally drying to a thickness of about five to seven thousandths (0.005 to 0.007) of an inch, treating different colored touching portions of the wet printed pattern simultaneously with a fog of spruce wood flour of which not more than a trace remains on a one hundred (100) mesh screen, fifteen to twenty-five percent (15 to 25%) remains on a two hundred (200) mesh screen and thirty-five to forty-five percent (35 to 45%) remains on a three hundred twenty-five (325) mesh screen, to produce a light application of said flour thereto to set the surface thereof, moving the resulting treated base through 25 a loop path with the treated face inside with wood flour of the above mentioned kind in said loop, brushing very lightly the surface with the wood flour thereon to move said wood flour into said paint and remove excess wood flour from said surface, drying said wet print paint, and abrading excess wood flour from the surface of the dry print paint.

4. The method of making ornamental printed felt base covering material, which consists essentially in printing a pattern of different touching colors onto a suitably prepared felt base backing with print paint, treating different colored touching portions of the wet printed pattern simultaneously to produce a light application of very fine wood flour of suitable color to the surface of said printed paint to "set" said surface, treating different colored touching portions of the "set" surface simultaneously to a heavier application of said wood flour, moving said wood flour into said paint and removing excess thereof from said surface, drying said wet print paint, removing excess wood flour from the surface of the dry print paint, and applying a protective coating to the resulting surface.

5. The method of applying an ornamental surface to a backing comprising applying print paint to said backing, characterized by sliding a mass of wood flour relatively over the surface of the applied print paint while said surface is still wet to cause wood flour to be picked up from said mass by the wet paint.

6. The method of applying an ornamental surface to a backing comprising applying print paint to said backing, characterized by moving said printed backing while said printed paint is still wet through a loop path with the printed face inside with wood flour in said loop to cause the printed face moving relatively to and in contact with the wood flour to pick up and retain wood flour.

7. The method of applying an ornamental surface to a backing comprising applying print paint to said backing, characterized by subjecting the surface of the applied print paint while it is still wet to a light application of wood flour and then to a heavier application thereof.

8. The method of applying an ornamental surface to a backing comprising applying print paint to said backing, characterized by subjecting the surface of the applied print paint while it is still

wet to a fog of wood flour and then to an undispersed mass of wood flour.

9. The method of modifying on felt base covering material the appearance of a print paint coating of differently colored touching areas which provide a pattern, comprising forming a loop of said material with said print paint coating inside said loop and while said coating is still wet, applying finely divided wood flour in said loop over said differently colored areas while said 5 10

print paint coating is still wet, moving said material while maintaining said loop to cause said wood flour to become incorporated in said coating, and removing excess wood flour from the surface of said coating.

SAMUEL A. COHEN.

RICHARD L. NEWMAN.

THOMAS LEONARD MORRILL, JR.

CHARLES D. THURMOND.